

1

3,561,152

## BIOCIDAL FUEL COMPOSITIONS

Roman W. Kulow, Cheshire, Conn., assignor to Olin Corporation, a corporation of Virginia  
No Drawing. Filed Mar. 4, 1968, Ser. No. 709,958  
Int. Cl. C10I 1/24

U.S. Cl. 44—63

8 Claims

### ABSTRACT OF THE DISCLOSURE

Biocidal fuel compositions have been disclosed which comprise a liquid hydrocarbon fuel containing a biocidally effective amount of selected amine salts of 2-mercaptopypyridine-1-oxide.

This invention relates to biocidal fuel compositions, and more particularly, to fuel compositions containing selected amine salts of 2-mercaptopypyridine-1-oxide.

It is known that microorganisms subsist in fuel systems, contributing to a variety of problems with respect to both storage and use of the fuel. Thus, microorganisms emulsify fuel and water forming slimes, generally at the fuel-water interface, which interfere with subsequent use of the fuel.

While this problem of microbial contamination is found in all fuel systems, it is particularly acute in aviation fuels, where, as disclosed by J. M. Sharpley in Elementary Petroleum Microbiology, Gulf Publishing Co., Houston, Tex. (1966) pp. 58-62, the fungus *Cladosporium resinae* is the most prevalent microorganism. It is readily apparent that slimes in aviation fuels will plug filters and other equipment, thereby increasing maintenance expenditures and jeopardizing normal aircraft operations.

Exclusion of moisture from fuel systems is impractical, and thus biocides, i.e., materials which kill microorganisms and/or inhibit their growth, must be used. Such biocides must fulfill many critical requirements. Thus, in addition to possessing the required biocidal activity, they must exhibit no deleterious effects on the fuel properties. Furthermore, they must not corrode storage tanks or fuel system equipment.

Now it has been found that fuel compositions containing, as biocidal agents, selected amine salts of 2-mercaptopypyridine-1-oxide are effective in inhibiting growth of microorganisms in fuel systems. The biocidal agents employed in this invention have the formula



wherin R is hydrogen or an alkyl moiety having 1 to 18 carbon atoms and R' is an alkyl moiety having 3 to 18 carbon atoms.

These amine salts I are readily provided according to the process described in U.S. Pat. 2,742,393 by reacting an appropriate amine with 2-mercaptopypyridine-1-oxide in a substantially anhydrous organic solvent. The reaction is exothermic, and temperatures between about 0° and about 60° C. are preferably maintained.

Illustrative amines which can be employed in the preparation of the amine salts I utilized in this invention include primary amines such as isopropylamine, t-butylamine, hexylamine, heptylamine, octylamine, nonylamine, decylamine, laurylamine, stearylamine and isomers thereof. Secondary amines such as diisopropylamine, dibutylamine, dioctylamine, n-propyl-t-butylamine, pentylhexyl-

2

amine, n-propylaurylamine, and the like can also be employed herein.

While any compound having the Formula I can be suitably employed in the practice of this invention, preferred embodiments utilize those amine salts I wherein R is hydrogen and R' is alkyl having 3-14 carbon atoms or R is alkyl having 1-6 carbon atoms and R' is alkyl having 3-6 carbon atoms.

Any liquid hydrocarbon fuel can be protected against microbial contamination according to the teaching of this invention. Exemplificative fuels which comprise kerosene-grade petroleum fractions include No. 2 fuel oils as defined in ASTM Tentative Specification D-396-64T and aviation turbine fuel as defined in Tentative Specification D-1655-65T of the ASTM Standards on Petroleum Products.

While the biocidal effect of amine salt I in fuel systems is observed over a wide range of biocide concentration, generally from .1 to about 5 p.p.m., and preferably from about .5 to about 2 p.p.m. of the biocide is employed. Greater and lesser amounts can be utilized, and the ranges set forth herein are not intended to be limiting.

In accordance with the practice of this invention, the biocidal agents I can be incorporated in fuels in many different ways. Thus, they are added to the fuel at any point, for example either prior to, during or after filling of a fuel tank. It is also feasible to supply the biocides to the fuel in the form of solutions or suspension in a portion of fresh fuel. Solvents, diluents, antioxidants and other ingredients can be advantageously admixed with the biocide prior to incorporation in the fuel system.

The effectiveness of the biocidal fuel compositions of this invention is particularly surprising and unexpected in view of the ineffectiveness of various other materials derived from 2-mercaptopypyridine-1-oxide in this application. Thus, while it is known that 2-mercaptopypyridine-1-oxide and its derivatives possess biocidal activity, it has been found that such derivatives as the ammonium salt of 2-mercaptopypyridine-1-oxide and disulfide derivatives such as 2,2'-dithiopyridine-1,1'-dioxide are ineffective in inhibiting growth in fuel systems.

The following examples will serve to illustrate the process of this invention.

### EXAMPLE 1

#### (A) Preparation of t-butylaminesalt of 2-mercaptopypyridine-1-oxide

A solution of 48.3 g. (0.38 mole) of 2-mercaptopypyridine-1-oxide in 475 ml. of chloroform was dried over 50 g. of anhydrous sodium sulfate. A total of 31 g. of t-butylamine was added dropwise, with stirring, to the 2-mercaptopypyridine-1-oxide solution over a 20 minute period. A reaction temperature of 10-15° C. was maintained during the addition. Filtration of the reaction mixture provided a solid product which was vacuum dried at 30° C./29 in. Hg to yield 45.7 g. of the t-butylamine salt of 2-mercaptopypyridine-1-oxide, M.P. 167-170° C.

#### (B) Preparation and testing of fuel composition

The t-butylamine salt of 2-mercaptopypyridine-1-oxide described in Part A was added in varying amounts to a number of 750 ml. portions of kerosene. Each of the resulting compositions was then mixed in a separatory funnel with 30 ml. of water containing *Cladosporium resinae* ( $10^6$  organisms/ml.). The flasks were stoppered, stored at room temperature and shaken several times per day. At intervals, aliquots were taken from both the kerosene and the aqueous phase of each mixture, streaked on agar and then incubated at 37° C. for 96 hours. At the end of the incubation period, the samples were examined and rated 0 for sterility or + for growth. The results of the tests are set forth in the table below.

**3**  
**EXAMPLE 2**

(A) Preparation of diisopropylamine salt of 2-mercaptopypyridine-1-oxide

To a solution of 25.4 g. (0.2 mole) of 2-mercaptopypyridine-1-oxide in 100 ml. of chloroform was added gradually, with stirring, at 10-15° C., 20.2 g. (0.2 mole) of diisopropylamine. After stirring the reaction mixture for one hour, chloroform was removed on a rotary film evaporator, thereby providing 31 g. of the diisopropylamine salt of 2-mercaptopypyridine-1-oxide, M.P. 94-96° C.

(B) Preparation and testing of fuel compositions

Following the procedure of Example 1, compositions were prepared and tested employing the diisopropylamine salt of 2-mercaptopypyridine-1-oxide as the biocide. The results are set forth in the table below.

**EXAMPLE 3**

(A) Preparation of laurylamine salt of 2-mercaptopypyridine-1-oxide

Laurylamine (72.8 g., 0.394 mole) was added, with stirring, in small portions to a slurry of 2-mercaptopypyridine-1-oxide (50 g., 0.394 mole) in 300 ml. water and 100 ml. ethanol at room temperature. When the addition was completed, the resulting solution was filtered and evaporated in a rotary evaporator at 70-80° C./20-30 mm. Hg to provide a light colored solid. Drying of the solid product for an additional 16 hours under vacuum yielded 103 g. of the laurylamine salt of 2-mercaptopypyridine-1-oxide, M.P. 80-81° C.

(B) Preparation and testing of fuel compositions

Following the procedure of the previous examples, compositions were prepared and tested employing the laurylamine salt of 2-mercaptopypyridine-1-oxide as the biocide. The results are set forth in the table below.

**COMPARATIVE EXAMPLES 1-3**

For purposes of comparison, fuel compositions were formulated and tested as described in the previous examples employing the following biocides:

C-1: Control (no biocide)

C-2: Ammonium salt of 2-mercaptopypyridine-1-oxide (prepared according to U.S. Pat. 2,686,786, Example 12)

C-3: 2,2'-dithiopyridine-1,1'-dioxide (prepared according to U.S. Pat. 2,742,476, Example 1)

TABLE I

| Example: | Concentration<br>of biocide<br>(p.p.m.) | Time (days) |   |   |     |    |
|----------|-----------------------------------------|-------------|---|---|-----|----|
|          |                                         | 1           | 5 | 7 | 170 |    |
| 1.....   | 0.5                                     | 0           | 0 | 0 | 0   |    |
|          | 1.0                                     | 0           | 0 | 0 | 0   |    |
|          | 2.0                                     | 0           | 0 | 0 | 0   |    |
|          | 2.5                                     | 0           | 0 | 0 | 0   |    |
|          | 5.0                                     | 0           | 0 | 0 | 0   |    |
| 2.....   | 1.0                                     | 0           | 0 | 0 | 0   | 60 |
|          | 2.5                                     | 0           | 0 | 0 | 0   |    |
|          | 5.0                                     | 0           | 0 | 0 | 0   |    |
| 3.....   | 1.0                                     | 0           | 0 | 0 | 0   |    |
|          | 2.5                                     | 0           | 0 | 0 | 0   |    |
|          | 5.0                                     | 0           | 0 | 0 | 0   |    |
| C-1..... | 0                                       | +           | + | + | +   |    |
| C-2..... | 1.0                                     | +           | + | + | +   |    |
| C-3..... | 0.5                                     | +           | + | + | +   |    |

**4**  
**EXAMPLE 4**

The amount of 80 grams of the t-butylamine salt of 2. The fuel composition of claim 1 wherein from about tank of JP-4 jet fuel containing approximately 250 gallons of water. After 90 days at ambient conditions, no growth is observed.

What is claimed is:

1. A fuel composition which comprises a liquid hydrocarbon fuel containing a biocidally effective amount of 10 an amine salt having the formula



20 wherein R is hydrogen or an alkyl moiety having 1 to 18 carbon atoms and R' is an alkyl moiety having 3 to 18 carbon atoms.

2. The fuel composition of claim 1 wherein from about 25 0.1 to about 5 p.p.m. of said amine salt is employed.

3. The fuel composition of claim 1 wherein R is hydrogen and R' is an alkyl moiety having 3 to 14 carbon atoms.

4. The fuel composition of claim 3 wherein the t-30 butylbutylamine salt of 2-mercaptopypyridine-1-oxide is employed as the amine salt.

5. The fuel composition of claim 3 wherein the laurylamine salt of 2-mercaptopypyridine-1-oxide is employed as the amine salt.

35 6. The fuel composition of claim 1 wherein R is an alkyl moiety having 1 to 6 carbon atoms and R' is an alkyl moiety having 3 to 6 carbon atoms.

7. The fuel composition of claim 6 wherein the diisopropylamine salt of 2-mercaptopypyridine-1-oxide is employed as the amine salt.

40 8. A binary system comprising a liquid hydrocarbon fuel and water, said system containing a biocidally effective amount of an amine salt having the formula



55 wherein R is hydrogen or an alkyl moiety having 1 to 18 carbon atoms and R' is an alkyl moiety having 3 to 18 carbon atoms.

**References Cited**

**UNITED STATES PATENTS**

60 2,742,393 4/1956 Bernstein et al. ----- 424-308  
2,975,042 3/1961 Summers, Jr. ----- 44-78  
2,975,043 3/1961 Ambrose ----- 44-78

DANIEL E. WYMAN, Primary Examiner

65 Y. H. SMITH, Assistant Examiner